

Jan. 30, 1951

F. A. J. VAN HALL, ET AL  
PROCESS FOR THE INTENSIVE AFTERTREATMENT  
OF SYNTHETIC THREADS

2,539,980

Filed April 1, 1948

3 Sheets-Sheet 1

Fig. 1.



Floris Adriana Jan van Hall  
and Daniel Rogla Barcelo

334

Albin F. Knight

Attorney

Jan. 30, 1951

F. A. J. VAN HALL ET AL  
PROCESS FOR THE INTENSIVE AFTERTREATMENT  
OF SYNTHETIC THREADS

2,539,980

Filed April 1, 1948

3 Sheets-Sheet 2



Inventors  
Floris Adriaan Jan van Hall  
and Daniel Rogla Barcelo

Albin F. Knight  
Attorney

Jan. 30, 1951

F. A. J. VAN HALL ET AL  
PROCESS FOR THE INTENSIVE AFTERTREATMENT  
OF SYNTHETIC THREADS

2,539,980

Filed April 1, 1948

3 Sheets-Sheet 3

*Fig. 4.*



*Fig. 6.*



*Fig. 5.*



*Fig. 9.*



*Fig. 8.*



Inventors

Floris Adriaan Jan van Hall  
and Daniel Rogla Barcelo

334

Alvin F. Knight  
Attorney

## UNITED STATES PATENT OFFICE

2,539,980

## PROCESS FOR THE INTENSIVE AFTER-TREATMENT OF SYNTHETIC THREADS

Floris Adriaan Jan van Hall and Daniel Rogla  
Barcelo, Barcelona, Spain, assignors to American Enka Corporation, Enka, N. C., a corporation of Delaware

Application April 1, 1948, Serial No. 18,408  
In Spain April 12, 1947

2 Claims. (Cl. 18—54)

1

This invention relates to the manufacture of synthetic threads according to the wet spinning method and more particularly to a process for the liquid treatment of a linearly moving thread. More specifically the invention concerns the effecting of after treatments with different treating liquids sequentially on continuously moving threads.

When manufacturing rayon according to the wet spinning process, the spinning solution, for example viscose, is extruded by means of a spinneret into a spin bath. The thread formed therein is coagulated and partially regenerated in the spin bath or the regeneration may be substantially completed in a complementary second bath. During the treatment in the second bath, while the thread is being decomposed into cellulose hydrate, a stretching operation is often applied. Finally, the thread is wound on bobbins or collected in a centrifugal bucket.

In this customary process the thread, after being collected on bobbins or in cakes, must be submitted to after treatments in order to remove the residual salts and impurities deposited during the manufacturing process. These treatments comprise deacidifying, bleaching, washing, and finally, drying.

Although the above referred to standard process has been developed to a highly efficient point, certain disadvantages are still present therein.

Certain disadvantages of the standard process are found to occur in the liquid after treatments. Additionally the process is objectionable in that during the formation of the thread package, irregularities occur in the thread. This is inherent in the process for the reason that it is practically impossible to coagulate and after treat all parts of the thread under the same conditions. The action of the after treatment baths is not uniform throughout all portions of the package, particularly in the extreme interior and exterior portions thereof. During the drying of the packages as normally produced and treated, differences in tension are created within the packages which effect different degrees of contraction therein and cause irregularities to exist in the final products.

In an effort to improve the physical and chemical properties of the thread, the synthetic textile industry has resorted to what is known as continuous spinning, and various schemes have been proposed to pass the thread continuously through the different baths for coagulation and after treatment. Some of these processes are based upon the immersion of the thread in successive

reservoirs containing the desired liquids; others are based upon the wetting of the thread as it is passed over a number of complicated rotatable reels which are operated in such a manner as to cause the thread to progress axially of the reels in a multiplicity of convolutions. Another process involves the treatment of the thread while it is passed axially of two angularly disposed cylinders, means being provided to apply the particular treating liquid to each of the respective sets of cylinders and the arrangements being such that the liquids are moved in a direction opposite to the direction of progression of the thread convolutions. Means are further provided to maintain the treating liquids separate after the application thereof to the thread.

A more recent proposal involves liquid sprays which are projected onto the thread at an angle by means of a power nozzle. The thread to be thus treated passes upwardly between two driven godets and the nozzles are formed with thread guiding grooves, the walls of which bear against the thread adjacent the point of projection of the liquid thereon. This proposal is ineffective for a number of reasons. To maintain the thread against the walls of the guides as the liquid is projected thereon requires that the thread in traveling upwardly at an angle to the vertical be under high tension. The liquid which is projected upon the thread at an angle as it is thus propelled under high tension largely falls away and has little effect on the thread. Due to the tension, the liquid will not have ready access to the individual filaments of the thread bundle and it will not properly penetrate and treat the same. Additionally the walls of the guiding groove contacted by the thread prevent the liquid from filming and forming a substantial sheath around the periphery of the thread. All of these factors tend to defeat the purpose of the treatment, and the effect of such of the liquid as is retained by the thread is limited.

All of the former processes proposed for solving the problems encountered in this art are of a more or less complicated nature and require a large and expensive plant, both from the standpoint of construction and maintenance. On the contrary, the present process is characterized by its great simplicity, since it eliminates the necessity for employing complicated mechanism. Furthermore, standard rayon manufacturing machines may be adapted for the new process with very little modification.

This novel process is based upon the surprising observation that the action of a treating liq-

2

uid upon a moving thread becomes extraordinarily intensive under certain conditions, under which conditions the treating liquid penetrates and surrounds the component filaments of the thread bundle. These conditions may be summarized as follows:

1. The thread must be entirely free of any contact with any thread guides, supporting members, or other elements of the spinning machine which tend to hold the individual filament thereof in tight association from the point where the liquid contacts the thread to the treatment bath from which the thread emerges.
2. The liquid should be applied to the thread at an extreme point in its upward path of travel, i. e., the ascending thread is contacted with a stream of liquid moving in a counter-current direction.
3. The filaments constituting the thread must be untwisted and in parallel relationship.
4. The thread must be under a low tension.
5. The thread must ascend in a substantially vertical path.

If the above conditions are met, the liquid surrounds the thread in the form of a sheath and penetrates between the individual filaments. The thread takes a very characteristic shape in the path of treatment, namely, the thread appears to be many times thicker, which is apparently due to the adherence and absorption of the liquid thereon, causing an intensive swelling of the thread. Under these circumstances the action of the treating liquid is rendered much more rapid and effective, so that when the thread moves at a speed of over 60 meters per minute, the thread's vertical path does not have to exceed 70 cm. in order to realize a complete coagulation, desulphurization or other desired treatment. The reaction speed is attributed to the fact that the contact surface of the thread, or better said, of the elementary filaments, with the liquid is at a maximum.

Provided the above set forth conditions are strictly adhered to, this intensive action of the liquid is equally striking in various kinds of after treatments, such as in the removal of salts, deacidification, washing, desulphurization, possibly removal of copper, bleaching, anti-chlorine treatment, and different types of finishing operations. In effecting the several different after treatments in a continuous operation the jets or streams of the liquids are applied successively, the treatments normally corresponding to the respective bath treatments utilized in the production of the particular synthetic thread involved in the various commercial operations.

The liquid treatment step of the invention may be utilized in any system or operation where it is desired to intensively treat a vertically ascending thread, and whereas many modifications can be made in the different forms of apparatus utilized, the invention can be more fully understood by reference to the accompanying drawings, wherein:

Figure 1 is a schematic illustration in side elevation of one particular type of continuous spinning machine constructed in accordance with this invention in which the treating troughs and ring twisting device are shown in cross-section;

Figure 2 is a schematic view in perspective illustrating a liquid treating system constructed in accordance with this invention including the system for re-circulating the treating liquid in its relationship to the thread;

Figure 3 is a detailed illustration of the mechanism intended to be used in the adjustments of the guiding rollers which control the spacing of the thread convolutions upon the driven rollers shown in the upper portion of Figure 1;

Figure 4 is a side elevational view of one of the liquid vessels provided with a depending liquid jet forming spout constructed in accordance with this invention which has been found to be particularly suitable for use in the process, the manner in which the thread is enveloped with a sheath of liquid as it is passed upwardly within the space defined by the spout being illustrated;

Figure 5 is a top plan view of the structure illustrated in Figure 4;

Figure 6 is an end view of the structure illustrated in Figure 4;

Figure 7 is a side elevational view of another type of liquid vessel and spout similar in purpose to the structure shown in Figure 4;

Figure 8 is a top plan view of the structure illustrated in Figure 7; and

Figure 9 is an end view of the structure illustrated in Figure 7.

In referring to the drawings in detail the thread or filament which is formed and after treated in the apparatus shown in Figure 1 is indicated at 10. Thread 10 is formed by the extrusion of a spinning solution through a spinneret 11 into a spin bath contained in trough 12. The thread is led from the spin bath through a thread guide 13 to a driven roller 14. Thereafter the thread is passed to a small freely rotatable roller 15 following which it is wrapped several times around the two rollers. A roller 16 is mounted for free rotation within a collecting trough 17 positioned adjacent to and in the same plane as trough 12. Roller 16 is utilized as a lower guide for the thread. The thread is passed to and around roller 16 from roller 14 and then upwardly to driven roller 18 which is of larger diameter than roller 14. Roller 18 is driven at the same R. P. M. by the same shaft (not shown) that drives roller 14.

Due to the arrangement described the thread is stretched in its passage from roller 14 around roller 16 to roller 18.

A series of rollers 19, 20, 21 and 22 are axially aligned with rollers 14 and 18 and are driven by the same shaft. These rollers 19, 20, 21 and 22 are therefore rotated together with rollers 14 and 18 and they are of the same diameter as roller 18. Consequently, the peripheral speeds of the rollers 18, 19, 20, 21 and 22 are the same. Arranged directly below each of the rollers 19, 20, 21 and 22 are collecting troughs 23, 24, 25 and 26, respectively. These collecting troughs are arranged adjacent to trough 17 in the same horizontal plane and the walls constituting the partitions for separating the troughs are designated as 27, 28, 29 and 30. A roller similar to roller 16 is mounted for free rotation in each of the collecting troughs 23, 24, 25 and 26, these rollers being designated as 31, 32, 33 and 34, respectively.

After the thread 10 has been passed to roller 18 it is passed to a freely rotating elongate roller 35 in axial alignment with roller 15 and it is then wrapped several times around rollers 18 and 35. Thread 10, after leaving roller 18, is passed around roller 31 in collecting trough 23 and thence upwardly around roller 19, after which it is wrapped several times around rollers 35 and 19 before passing downwardly around

roller 32 in collecting trough 24. As the thread progresses through the machine it is led upwardly from roller 32 around roller 20 and then several wraps of the thread are made around roller 35 and roller 20 before the thread is again passed downwardly to a point where it is led around roller 33 in collecting trough 25. In order to effect additional treatments of the thread it is passed upwardly from roller 33 and wrapped several times around roller 21 and 10 roller 35, after which it is passed around roller 34 in the last of the troughs illustrated and then upwardly and around roller 22.

In the liquid treatment section of the apparatus as thus described, the thread 10 in its upward flight passes substantially vertically to rollers 19, 20, 21 and 22, respectively. During each of the upward flights of the thread a treating liquid is supplied thereto by means of liquid vessels provided with spouts, the vessels being designated as 36, 37, 38 and 39, respectively. A similar vessel 40 may be utilized to supply liquid to the thread passing upwardly from roller 16 but for the reasons hereinafter discussed any suitable means for supplying a liquid to a moving thread may be utilized at this position. The vessels 36-40, inclusive, may be of the form illustrated in Figures 4-9, inclusive, although it has been found that the vessel illustrated in Figures 4-6, inclusive, is particularly well adapted for use as the treating vessel at 36, 37, 38 and 40. On the other hand, the vessel illustrated in Figures 7-9, inclusive, is particularly suited to be the treating vessel at 39.

The single vessel 36 and its circulation system are illustrated in Figure 2 and are exemplary of the remaining vessels and their associated systems illustrated in Figure 1. Vessel 36 is formed with an upstanding cup portion 41 from the upper portion of which extends an elongated lip or spout 42. Lip 42 is arcuate in transverse cross-section and for a considerable portion of its length upwardly from its lower tip it is arranged in a plane parallel to the path of travel of thread 10 in its upward flight. The lip or spout 42 is made arcuate in cross-section so as to partially encircle the thread for applying to the thread a counter-current moving sheath or envelope of treating liquid as the thread passes upwardly therethrough.

In Figure 2 the thread is shown in a single vertical flight in association with the roller 31 positioned in trough 23. The recirculating system includes a liquid reservoir 43. Treating liquid is fed from the reservoir through pipe 44 provided with a cock 45 for controlling or shutting off the supply as desired. Cup portion 41 is maintained in a fixed but adjustable position near the upwardly moving thread by means of a support 46 and a bracket 47. In use, the liquid is fed to the vessel 41 at a predetermined rate and it overflows the depressed edge of the cup portion and passes downwardly within the spout or lip 42 in the form of a gentle stream through which the ascending thread moves. Since the liquid surrounds the thread in its upward passage as an envelope or sheath, the thread is maintained in proper position with respect to the spout. The thread is propelled at a speed such that the treating liquid will flow counter-current thereto as the liquid is carried downwardly by gravity. The liquid will collect in trough 23. The recirculation of the liquid may be so regulated that the trough contains a

liquid bath at a level above roller 31 as illustrated in the drawings. The liquid in each of the circulating systems is of the desired chemical composition, depending upon the particular treatment there preferred, and it is maintained uniform so that uniformity will be had in all parts of the thread as it is continuously treated in the particular operation. The thread in its vertical flight should be free of contact with guides below the vessel or immediately thereabove, that is, any guide employed above the vessel should be of such a nature as to avoid the closing of the thread and the pressing of the treating liquid therefrom.

The liquid in trough 23 may be continuously recirculated by being propelled through a pipeline 48, valve 49 to tank 43. The liquid during recirculation may be purified and regenerated as is desired or necessary.

Thread 10 being propelled upwardly within the lip or spout 42 is passed so that it will not be damaged or closed by pressure from the wall of the lip or spout.

Referring now again to Figure 1, the thread 10, after having been passed through the liquid treating steps in the apparatus is directed to roller 50 and then around a drying roller 51. It is then passed to elongate, freely rotatable roller 52 and wrapped several times around the rollers 51 and 52. Roller 51 which is utilized as a drying roller is frusto-conical in form to permit the contraction of the thread as it is passed over the two rollers. Roller 51 may be in the form of a cylinder and may be heated on the interior by any suitable means. The dried thread is passed from roller 51 downwardly through a thread guide 53 and then over a fier which slides over a ring 54. Ring 54 is mounted to be raised and lowered in the normal manner in order to control the winding pattern of threads laid up on bobbin 55. The ring twister is illustrated schematically in Figure 1 as being driven by an electric motor 56 which may be adjusted at two speeds. A slip clutch 57 of the centrifugal force type is provided which permits slip to the desired degree.

In Figure 3 a support is illustrated which may be utilized in adjusting rollers 15 and 35 with respect to rollers 14, 18, 19, 20, 21 and 22. The adjustment of this support will permit a change in the relative inclination of the axes of the two sets of rollers for the purpose of controlling the spacing of convolutions of the thread on the rollers. This is accomplished by pivoting shaft 58 which may support rollers 15 and 35 at 59 to bracket 60. Bracket 60 is fastened to the machine frame designated at 61. Adjustment screw 62 is threaded into pivoted nut 63 which in turn is secured to bracket 60, and the screw has its free end pivotally anchored at 64 to the end piece of shaft 58. Upon turning screw 62 by the wing head 65 shaft 58 will be caused to move about pivot 59 and accordingly adjust the inclination of the axis of rollers 15 and 35 toward or away from the axis of rollers 14, 18, 19, 20, 21 and 22 to the desired degree. The shaft for roller 52 may be similarly mounted for adjustment.

It is to be noted that the thread, as illustrated in Figure 1, as it is propelled to and from the rollers 31, 32, 33 and 34 is passed around the driven rollers 18, 19, 20, 21 and 22, respectively, and that these latter rollers are coaxial and are of the same diameter. Accordingly the thread as it is moved during these liquid treatments is under substantially no tension. As

has been previously pointed out, this is one of the conditions that is considered essential in order to effect the intensive treatment of the thread contemplated by this invention. It is for this reason that it has been stated that any means suitable for applying liquid to the thread passing from roller 16 to roller 18 will be sufficient since the thread during such passage is under high tension due to the difference in the diameters of rollers 14 and 18. However, in an operation in which stretching of the thread is not effected at this stage of the process, a vessel of the type contemplated by this invention may be utilized with the same efficient results as are had in the remaining steps in which the thread is passed under substantially no tension.

It has also been found possible under certain conditions to effect more than one treatment of the thread within one ascending path of travel. This may be accomplished by positioning two of the liquid vessels one above the other in the aforesaid relationship to the thread. In such an operation the treating liquids must be such as will permit the mixture thereof. It has been found feasible when it is desired in the production of viscose yarn to finish the thread immediately after desulphurization. In such an operation, therefore, the liquid vessel for applying the finishing liquid may be disposed in the upper portion of the thread flight and the liquid treating vessel for the washing operation may be positioned between the first vessel and the bath trough located vertically therebelow. Therefore in such operation the thread containing the desulphurizing agent is washed before it is subjected to the action of the finishing agent.

The treating vessel illustrated in Figures 4-6, inclusive, is formed with a supporting bar 66 which is adapted to be clamped in a bracket mounted on the machine. The upstanding cup is illustrated at 67 and a depending lip or spout 68 merges with the cup at 69 below the upper surface of the cup. The inner portion 70 of the spout extends parallel to the cup portion 67. The cup portion 67 has a conical lower end 71 on which is provided a connection 72 for the reception of a flexible tube or other suitable liquid conductor. Spaced guides 73 extend outwardly over and beyond the spout from the upper edge of the cup portion 67 and these guides are so spaced that they tend to line up the thread upon any tendency of the same to jump beyond the edges of the walls 74 of the spout. The construction is such that the overflowing treating liquid is gently directed downwardly counter-current to the passage of the thread and the spout is so constructed that the thread is opened and placed in a liquid sheath or envelope. This application of the liquid tends to draw the individual filaments apart and permit ready access of the counter-flowing liquid to each of the individual filaments of the upwardly moving thread. The nature of the curve of the wall of the spout is such that the liquid stream is caused to assume a form which will envelope and impregnate the thread without any tendency to press out the liquid or close the thread as it passes within the spout.

The vessel illustrated in Figures 7-9, inclusive, is formed with a supporting rod 75 which may be mounted in the same manner as that of the vessel illustrated in Figures 4-6, inclusive. This vessel is provided with a downwardly extending coni-

cal spout 76 which has an opening 77 vertically extending throughout its height. A connection for a flexible hose or other liquid supply conductor is illustrated at 78 and the liquid supplied through the conductor will accumulate in the conical spout 76. The liquid in the conical spout will form a sheath or envelope upon the thread when it is passed through the center of the spout. Opening 77 is utilized in threading up the machine. In the construction illustrated in Figures 7-9, inclusive, the thread is not readily displaced from the spout and a uniform operation may be had without encountering any tendency to close the thread by contact with the walls of the spout as the thread passes upwardly in counter-current movement with respect to the treating liquid.

The execution of the process to which the present application relates will be understood better by means of the following examples:

#### Example I

A normal viscose spinning solution with 6% cellulose and 7% NaOH was coagulated in a sulphuric acid bath of 7%  $H_2SO_4$  containing zinc salt and sodium salt and having a specific gravity of 1.3 at 20° C. This thread was subjected to a preliminary stretch treatment between the spinneret 11 and the roller 18. Dilute sulphuric acid of 3% concentration at a temperature of about 85° C. was applied to the thread by the vessel 40 in the flight leading upwardly to the roller 18. (The effect of the dilute sulphuric acid is that of de-xanthating and coagulation, while swelling is produced in the bath within the tank 17.) At vessel 36 the thread was treated with pure water at a temperature of about 80° C. and at vessel 31 it was subjected to a desulphurizing treatment by a solution of 1.5% sodium sulphide. At vessel 38 it was subjected to another washing treatment with water at a temperature of about 80° C. and finally, at vessel 39, it was supplied with an emulsion of 2% of a half-saponified fat. Thereafter the thread was passed to the drying cylinder 51 which was maintained at a temperature of 125° C. at a peripheral end speed of 50 meters a minute. With 20 turns along the cylinder 51, a wholly finished thread having a high degree of uniformity of physical and chemical properties was produced.

The dry thread issuing from the drying cylinder 51 was passed through the thread guide 53, flier 54, and onto bobbin 55 for twisting. As the high speed at which the twisting spindle of bobbin 55 normally rotates presents difficulties when threading onto the ring, the motor 25 may be driven at two speeds—the required take-up speed and the decreased speed used for threading up.

#### Example II

Normal viscose prepared from cellulose having a low hemi-cellulose content was spun through normal spinnerets into a Muller bath to form 1100 denier rayon having 275 filaments. After leaving the spin bath, the thread was guided in a substantially vertical direction alternately over draw off rollers and through treating baths, and during each ascending passage the thread was subjected to the treatment with liquids by means of the liquid treating devices shown in the drawings, and then dried, twisted, and collected, as shown therein. In the first path of thread travel to roller 18 a 3% sulphuric acid solution at 85° C. was applied to the thread. During the subsequent steps of the after treatment

the thread was treated respectively with water at 80° C., 1.5% sodium sulphide solution, water at 80° C., and finally a 2% finishing solution at vessels 36, 37, 38 and 39, respectively.

During each treatment the thread never deviated over 3° from the vertical. The length of path travel, that is, from the bath to the liquid treating device, was approximately 80 cm. The quantity of liquid supplied from each of the liquid treating devices was 600 cm.<sup>3</sup> per minute. Under these conditions the treatments were effected successfully and without any mishaps. The dried and twisted thread was neutral, had a high strength and could be used satisfactorily as tire yarn.

The process according to the invention, is not limited to the production of viscose rayon, as it is applicable to the spinning of any type of synthetic thread which may be spun according to the so-called "wet spinning" method wherein a series of liquid treating baths are employed. It is only essential that care be taken that an untwisted thread is passing under low tension through a substantially vertical path, and in this path the thread must not be in contact with any parts of the apparatus such as thread guides, rollers, etc.

What is claimed is:

1. In a method of intensively treating freshly spun synthetic threads according to the wet spinning process in which a spinning solution is extruded through a spinneret into a coagulating bath to form a thread consisting of a plurality of untwisted filaments and in which the thread is after treated and collected, the step which comprises propelling the thread in an upward direction in a substantially vertical path between two widely spaced guiding points while under a tension insufficient to effect a stretching thereof, and in the upper portion of the thread path during its ascending passage between said points initially guiding a jet of after treating liquid into contact with the thread and for a relatively small portion of the thread path in counter-current relation to the direction of the thread travel while avoiding any other contact of the thread between the guiding points whereby a

sheath of treating liquid envelopes the thread at the point of contact and moves downwardly along the thread during the major portions of its travel in the path and penetrates the individual filaments.

- 5 2. In a method of intensively treating freshly spun synthetic threads according to the wet spinning process in which a spinning solution is extruded through a spinneret into a coagulating bath to form a thread consisting of a plurality of untwisted filaments and in which the thread is after treated and collected, the steps which comprise propelling the thread in an upward direction in a substantially vertical path between two widely spaced guiding points while under a tension insufficient to effect a stretching thereof, and in the upper portion of the thread path during its ascending passage between said points initially guiding a jet of after treating liquid into contact with the thread and for a relatively small portion of the thread path in counter-current relation to the direction of the thread travel while avoiding any other contact of the thread between the guiding points, the movement of the thread being at such a speed that a sheath of treating liquid envelopes the thread at the point of contact and moves downwardly therealong to the lower end of the thread path thereby penetrating the individual filaments, collecting the treating liquid at the lower end of the thread path, and recycling the collected treating liquid.
- 10 30 FLORIS ADRIAAN JAN VAN HALL.  
DANIEL ROGLA BARCELO.

35

REFERENCES CITED

The following references are of record in the file of this patent:

40

UNITED STATES PATENTS

| Number    | Name                  | Date          |
|-----------|-----------------------|---------------|
| 2,317,152 | Costa et al. -----    | Apr. 20, 1943 |
| 2,351,110 | Davidson et al. ----- | June 13, 1944 |

45

FOREIGN PATENTS

| Number  | Country             | Date          |
|---------|---------------------|---------------|
| 515,127 | Great Britain ----- | Nov. 27, 1939 |